

## UNITED STATES PATENT OFFICE

KURT STÜRMER, OF PRUHLITZ, GERMANY

## PROCESS FOR TANNING ANIMAL HIDES WITH SALTS OF IRON

No Drawing. Application filed February 12, 1929, Serial No. 339,497, and in Germany February 18, 1928.

There is a known method of tanning animal hides by introducing divalent salts of iron (ferro salts) first into the fibre and by then oxidizing them into trivalent salts of iron (ferri salts)—which are to be deposited on the fibre—through treatment with higher nitric oxides  $N_2O_3NO_2$ , also with nitric acid. A process has also become known in which oxidation is carried out with a mixture of  $NO_2$  and  $NO$ , whereby compound salts of iron ( $FeSO_4O$ ) are formed.

All these processes have the disadvantage that the leather thereby obtained is brittle, as both  $NO_2$  and  $N_2O_3$ , like the nitric acid which is formed, immediately attack and finally destroy the fibre.

With this process, therefore, the gradual progress of oxidation cannot be regulated. Moreover, it is unavoidable that the top layers 20 of the hide should be over-tanned, and the complete tanning through the hide is only obtained at the expense of the grained surface being prejudicially affected. In addition to this, all the means of oxidation mentioned 25 cause the tanning-liquor to become very sour, so that after its application the leather takes on free acids at the same time which are "difficult or quite impossible to remove."

The above-mentioned disadvantages are entirely overcome in the process forming the 30 object of the present invention: In my process the raw hide, or skin, is laid in a solution of salts of iron or other suitable ferro salts, the nitrogen monoxide ( $NO$ ) is introduced, 35 whereby any additional oxygen must be avoided. The nitric monoxide must be practically free from higher nitric oxides. Only when the solution of the compound ferro salts has completely penetrated the skin, so 40 that the section is of uniform colour, do I begin to oxidize.

An important point in the process is that, in the first phase of the tanning, the formation 45 of higher nitric oxides, such as  $N_2O_3$ ,  $NO_2$ ,  $HN_2O_2$ ,  $HNO_3$ , which always occur in the processes hitherto adopted, is avoided, and that nitric monoxide is used entirely alone. The dark violet solution of the com- 50 pound salts has the characteristic of being

absorbed by the animal fibre without attacking it in the slightest degree.

The raw hides or skins are first placed in sulphate of iron liquor of a definite concentration and after some time nitric monoxide 55  $NO$ , which must not contain any higher nitric oxides, is introduced into the liquor, whereby the above-mentioned compound salts are formed, which are very thoroughly and uniformly absorbed by the animal fibre. If the 60 raw hides or skins so treated are then treated with oxygen—by simply blowing air against them or adding oxygen under pressure—the fibre will be tanned in a surprisingly uniform and thorough manner.

The leather obtained in this way shows, in contradistinction to the kinds of leather hitherto obtained by iron tanning, a completely undamaged fibre, so that the leather is extremely tough, flexible and strong.

## Example

A solution of sulphate of iron with 180–400 g.  $FeSO_4 \cdot 7H_2O$  to the litre is treated with 75 nitric monoxide which is practically free from higher nitric oxides (no air being admitted) until no more  $NO$  is absorbed.

The quantity varies according to the temperature and concentration of the solution or the pressure of the nitric monoxide. It is 80 sufficient if about 1 cubic metre of  $NO$  is absorbed in one cubic metre of fluid. In the solution thus prepared, the raw hides or skins from which the lime has been extracted are 85 quickly introduced, and, according to the thickness, are allowed to stand in the solution for 2–24 hours. They are then taken out and dried in the air and only washed after drying. The raw hides or skins can also be placed first in the iron liquor, the nitric monoxide 90 being in this case only introduced afterwards. For 100 kilos of hide 10–15 kilos of salts of iron (reckoned as  $Fe_2O_3$ ) are required.

Instead of sulphate of iron, other divalent salts of iron which absorb nitric monoxide 95 can be used, such as ferro chloride ( $FeCl_2$ ) or ferro acetate. The treatment with oxygen can also be extended for any desired period without damaging the fibre.

Having now described my invention, what 100

I claim and desire to secure by Letters Patent  
is:—

1. Process for tanning animal hides using basic salts of iron, consisting in treating the hides with a solution of divalent salts of iron, then introducing into the solution substantially pure nitric monoxide and then oxidizing the hides.
- 5 2. Process in accordance with claim 1, wherein the hides are first placed in the solution of ferro salts and then pure nitric monoxide introduced.
- 10 3. Process in accordance with claim 1 subjecting the treated hides to the action of air or oxygen under pressure.
- 15 4. A process for tanning animal hides consisting in treating the skins with a solution of divalent salts of iron, which has previously absorbed nitric monoxide.
- 20 5. A process as set forth in claim 4, consisting in first bringing the hides into the solution of ferro salts whereupon pure nitric monoxide is introduced.

In testimony whereof, I have signed my name to this specification at Berlin this 29th day of January, 1929.

KURT STÜRMER.

30

38

40

45

50

55

60

65